

J. E. DAVIDSON.  
CORNER BINDING.  
APPLICATION FILED FEB. 1, 1913.

1,087,530.

Patented Feb. 17, 1914.



Witnesses:

John H. Parker  
Alice H. Morrison

Testator:  
John E. Davidson  
Esq. Archibald Alexander Duke  
Atteys

# UNITED STATES PATENT OFFICE.

JOHN E. DAVIDSON, OF BOSTON, MASSACHUSETTS, ASSIGNOR OF ONE-THIRD TO  
AUTHUR N. HOOD, OF NEWTON, MASSACHUSETTS, AND ONE-THIRD TO JOHN T.  
NIGHTINGALE, OF BOSTON, MASSACHUSETTS.

## CORNER-BINDING.

1,087,530.

Specification of Letters Patent.

Patented Feb. 17, 1914.

Application filed February 1, 1913. Serial No. 745,581.

To all whom it may concern:

Be it known that I, JOHN E. DAVIDSON, a citizen of the Dominion of Canada, residing at Boston, county of Suffolk, State 5 of Massachusetts, have invented a certain new and useful Improvement in Corner Bindings, of which the following is a specification, reference being had therein to the accompanying drawings.

- 10 My invention relates to corner bindings which are used to protect and secure the meeting edges of sections of material which are joined together at an angle to each other, and is particularly intended to provide an 15 improved corner binding for protecting securing and reinforcing the corners of boxes and the like in which such qualities as lightness, strength and durability are especially desirable.
- 20 Many boxes such for example as tea boxes are made preferably from thin light material, generally wood. Others are made from laminated wood, that is sheets or veneers which are laid and secured together. 25 and which when properly constructed form a light and strong material for boxes. Such boxes made from thin light wood are however relatively weak, because of the difficulty of securing the relatively thin material together firmly and strongly at the corners. When the corners are secured with the aid of a strong corner binding which 30 protects and reinforces them, a strong light box is produced which is admirably adapted 35 for a large variety of uses. Especially is this the case when the sides of the box are formed from built-up veneers as hereinabove referred to.

My invention consists in a molded corner binding made from laminated wood having the grain of the various veneers or sheets arranged in crossed relation and secured together and permeated by cement, all as will be clearly understood from the following description taken in connection with the drawings, forming a part hereof.

The novel features of the invention are pointed out and clearly defined in the claims at the close of the specification.

50 In the drawings, Figure 1 is a perspective of a corner binding embodying my invention partly broken away for greater clearness. Fig. 2 is a perspective view showing in section the corner binding applied

to the corner of a box. Fig. 3 is a transverse section of a thicker and heavier corner binding embodying my invention. Fig. 4 is a transverse section of a strip of laminated material from which the corner binding is formed, before the same has been molded to shape.

The nature and character of a corner binding embodying this invention will be readily understood from a description of the way in which it is produced.

I first form a strip or sheet of laminated wood, which consists of two or more, preferably three, sheets or laminae which latter may be readily formed by the use of a veneer machine of well known construction, from 70 properly tempered bolts or logs of wood. A moist sheet as it comes from the log is placed on a table and coated with a rather heavy coating of cement; another sheet is then laid on the first one, preferably with 75 the grain of the wood in crossed relation to the grain of the first sheet. This second sheet is also coated with cement, and a third sheet is placed on top of the second sheet with the grain of the wood running parallel 80 with that of the first sheet. A strip thus built up is shown in cross-section in Fig. 4 and I have there designated the respective layers as 1, 2 and 3. From the moist sheets of wood which are thus built up or superimposed the one on the other a strip is cut of a width equal to the width required for a given corner binding, which is to be formed, and of a suitable length. This moist sheet is then subjected to heat and 90 pressure in a molding machine having co-operating convex and concave molds corresponding to the interior and exterior shape of the corner binding. The material is thus molded to the shape desired, such for example as shown Fig. 2. By the heat and pressure the cement is caused to permeate the wood and to secure the sheets or laminae firmly together. The strip is allowed to dry under the heat and pressure of the molds 100 and the cement becomes set and fixed.

The number of plies or sheets of wood employed may, as will be obvious, be increased if greater thickness or strength is desired, and the thickness of the sheets used may 105 also be varied in accordance with the result desired. In Figs. 1, 2 and 4 I have shown a corner binding composed of three laminae

or sheets, while in Fig. 3 the corner binding shown is composed of five sheets.

The corner binding strip will generally have a right angle interior shape in cross section as shown Figs. 2 and 3. Since the usual box to which such a corner strip is applied has what are termed square corners the interior of the corner binding forms a sharp angle as shown at 6 so that it will correspond with and accurately fit the sharp edge of the corner of the box formed by the sides thereof, while the exterior of the corner binding is curved at the corner as shown at 4.

It is important that the binding fit snugly and tightly over the corner of the box to which it is applied and so that the inner surface of the binding which overlies the meeting edges of the sides of the box will lie closely in contact with the said sides. This greatly increases the strength of the whole structure. It is also important that the exterior corner 4 should be rounded since this rounded shape very greatly increases the strength of the corner against crushing strains which would tend to break it down or crush it in and a rounded exterior as at 4 is for purposes of handling and the like much more desirable than a sharp exterior corner would be.

As hereinabove noted the compressed and molded sheets or laminae of wood are not only firmly united and secured together by cement but the cement permeates the wood under the heat and pressure of molding. When the moist built-up strip having cement between the layers is subjected to the molding operation the heat and pressure expels the moisture and the cement in large measure replaces it and then dries and becomes set and fixed, filling the interstices of the wood more or less completely. A corner binding strip thus formed is largely homogeneous and is different in character from the wood from which the sheets or veneer

are formed. It is much tougher and stronger than wood, will not split, crack or fracture so easily and will resist a much greater breaking or crushing strain.

The corner binding is preferably secured in position on the box corners by means of clenched staples 7, Fig. 2, although other equivalent securing devices as clenched nails or the like may be employed.

What I claim is:

1. A corner binding, for boxes or the like, consisting of a plurality of thin layers of wood, with the grain of the wood in the different layers in crossed relation, said layers being permeated with and bound together by cement and molded to form a right angular structure the interior of which is shaped longitudinally to fit closely the corner of a box.

2. A corner binding, for boxes or the like, consisting of a plurality of thin layers of wood, with the grain of the wood in the different layers in crossed relation, said layers being permeated with and bound together by cement and molded to form a right angular structure the interior of which is shaped longitudinally to fit closely the corner of a box, and the exterior of which structure has a rounded corner.

3. A corner binding, for boxes or the like, consisting of a plurality of thin layers of wood, with the grain of the wood in the different layers in crossed relation, said layers being permeated with and bound together by cement and molded to form a right angular structure the interior of which is a sharp right angle to fit closely the corner of a box, and the exterior of which structure has a rounded corner.

In testimony whereof I affix my signature, in presence of two witnesses.

JOHN E. DAVIDSON.

Witnesses:

WILLIAM A. MACLEOD,  
ALICE H. MORRISON.